

Feb. 7, 1933.

T. F. MOORE

1,896,783

ELASTIC FABRIC

Filed June 24, 1932

2 Sheets-Sheet 1



Fig. 3.

Fig. 4.



Fig. 2.

INVENTOR.  
Thomas F. Moore,  
BY  
Robert K. Randall,  
ATTORNEY.

Feb. 7, 1933.

T. F. MOORE

1,896,783

## ELASTIC FABRIC

Filed June 24, 1932

2 Sheets-Sheet 2



INVENTOR.  
Thomas F. Moore,  
Robert K. Randall,  
ATTORNEY.

## UNITED STATES PATENT OFFICE

THOMAS F. MOORE, OF WESTERLY, RHODE ISLAND, ASSIGNOR TO GEORGE C. MOORE COMPANY, OF WESTERLY, RHODE ISLAND, A CORPORATION OF RHODE ISLAND

## ELASTIC FABRIC

Application filed June 24, 1932. Serial No. 619,076.

The present application is a continuation in part of my prior application Serial No. 571,363, filed October 27, 1931, in so far as the contents of this present application have 5 been set forth in such earlier application.

The invention relates to elastic fabrics, and has as its object the provision of novel and improved elastic fabrics for use in the manufacture of corsets, girdles, and other similar 10 and related garments or articles designed to support and confine the part of the body upon which they are worn.

Elastic fabrics, as properly so-called, have their elasticity conferred through the inclusion 15 of component elements which are themselves elastic and capable of elongation, such as the vulcanized rubber cords widely used for this purpose, as distinguished from fabrics made of purely textile elements in which 20 a certain amount of yield is attained through pulling out or straightening the bends and undulations into which the elements are thrown by reason of their twist or their interengagement in forming the fabric. But all commercially successful elastic 25 fabrics hitherto devised and used have had capacity for contraction and subsequent stretching conferred through the use of elastic elements extending only in one direction, either in the direction of their length 30 or of their width, and never in both directions at once. Corsets, girdles, and the like articles made from such prior fabrics have been inherently incapable of accommodating 35 themselves closely to the body of the wearer when the portion of the wearer's body has been subjected to bending within the width of the garment, as at the waist and across the hips of the wearer of such a garment.

40 This is because these elastic fabrics, hitherto having a stretch in only one direction, have to be employed with the direction of stretch disposed circumferentially around the wearer's body, in order to attain the desired 45 confining effect. Being inelastic and incapable of elongation in a direction up and down the wearer's body, the upper and lower margins of the garment are forced to slip and slide over the wearer's body as the underlying 50 portions of the body become more or

less convex and hence lengthened or shortened in surface, and these marginal portions tend thereafter to remain in the undesired positions to which they have been thus pulled, destroying the smoothness of line of the garment and causing discomfort and embarrassment to the wearer, and requiring undesirable manual readjustment to restore them to place. Also, uncomfortable and unsightly 55 folds tend to be produced on the concave side of the bend in the garment, with the accompanying well-known and unsightly fault of having the garment gape away from the wearer's back when in a bending or sitting 60 position.

With the object of overcoming these well-known drawbacks, I have devised novel elastic fabrics which are capable of being stretched simultaneously both in the direction of 65 their length and in the direction of their width and of course in any intermediate direction or directions as well. These novel fabrics are capable of being used alone, or in combination with the known fabrics having stretch in one direction only, to make 70 supporting and confining garments which will hug the wearer's body at all points in their width and conform to the changing convex and concave outlines of the body without slipping or gaping of the marginal 75 portions, and without wrinkling or folding across portions of concave outlines, because they are capable of contraction and expansion widthwise in similar manner to the extension and contraction of the underlying 80 surfaces of the wearer's body.

Since these fabrics are used almost exclusively in the manufacture of corsets, girdles, and other articles designed to surround and confine a portion of the wearer's body, their 85 chief function is to contract about and thus press radially inward upon the surface which they surround. To perform this primary function, in both woven fabrics such as shown and described herein, and knitted fabrics 90 such as form the subject-matter of my co-pending application filed Jan. 29, 1932, Serial No. 589,612, the elastic elements entering into their makeup which provide for such radial 95 contraction of the garment (which is ordinary 100

narily longitudinal contraction of the fabric when woven), have to exert a fairly considerable degree of contractive effort. This may be achieved in any of the familiar ways known in the art, as by running the longitudinal elastic elements as tightly as possible in the weaving or otherwise making them operate near the limit of their stretch when in wear, or by making these elements of large diameter and hence powerful in their contraction, or by putting them in large numbers and close together, or by a combination of these and other methods.

On the other hand, and as concerns the transverse stretch, which is directed up and down the portion of the body confined by the garment, I have found that this transverse contractibility of such a two-way stretch fabric must not exceed in its strength the tendency of the marginal portions of the garment to cling to the skin or underlying surfaces, otherwise the marginal portions of the garment will not be permitted to stay in their intended places while the enclosed portions of the wearer's body assume a convex or concave realtion and the main purpose of the provision of transverse stretch will thus be defeated. In other words, the main specific function of the provision of transverse stretch is to permit the garment to become wider or narrower exactly as the underlying skin areas lengthen or contract, so that there will be no movement relative to the skin at the top and the bottom edges of the girdle. The requisite of the transverse stretch is that it shall yield to permit the garment to increase its vertical width, or height, wherever needed, so that these marginal portions shall not be forced to slip at the convex side of a bend; but at the same time there must be sufficient contractive effort to bring the garment into shape when the enclosed part of the body is again straightened out, and also, if desired, to take care of the fullness otherwise forming at the concave side of a bend. Thus, it will be apparent that the tendency of the garment to contract transversely must not exceed the tendency of the marginal portions to cling through friction to the points on the wearer's body at which they have been applied, and the tendency to cling is determined largely by the working tension or contractive effort of the elastic elements which create the tightness of the confining portion of the garment.

I have found that there is thus a definite requirement that the transverse contractive effort, or resistance to stretch up and down the wearer's body, must be substantially less than the longitudinal (or peripheral) contractive effort exerted as the garment is worn, otherwise the marginal portions of the girdle will slip just as in the prior one-way stretch fabric girdles, and require to be tugged into place following a bending posture

of the enclosed portions of the wearer's body. Like the grip of the garment, the transverse contractive force may be modified in several ways, as by inserting the transverse elastic elements with relatively low tension or otherwise making them operate in lightly stretched relation when worn, or by putting in less rubber either by reducing the diameter of these elements or the frequency of their insertion, or by combinations of these ways. While I do not intend to restrict myself to any definite ratio, other than that just indicated, I will state for purposes of illustration that a satisfactory ratio can be attained in a woven fabric, where warps and wefts of the same size rubber and of the same count per inch, (or even materially higher weft count per inch), are used, and other factors being equal, by inserting the covered rubber warp cords so that they will be about 50% extended as they lie in the normal contracted fabric, while the covered rubber weft cords will have a 20% extension as they lie in the fabric under the same conditions, with the warpwise and weftwise extension of the fabric as a whole limited respectively to around 50% and 30% above its contracted dimensions. The tensions thus given to the elastic warps and wefts are of course modified by the presence, number, and length of the non-elastic or fibrous warps generally used in all elastic fabrics, and the number, size, and length of the picks of the weft, both elastic and non-elastic, within limits known to those skilled in this art.

To fulfill the primary function of the fabric in making a confining garment, the rubber warps employed are preferably but not necessarily of fairly large diameter, the uncovered rubber core being on the order of 1/30 or 1/40 of an inch, whereas the rubber wefts are of much smaller diameter, their core frequently being of 1/100 of an inch in size, and in all cases being approximately commensurate with the size of the non-elastic warps and wefts which are or may be used in these fabrics; an elastic cord essentially suitable for use as weft in carrying the invention into effect is that set forth in U. S. Letters Patent #1,892,847, granted on Sept. 8, 1931 to Percy Adamson.

Under all ordinary circumstances, there will be a greater amount of rubber in the warp than in the weft, or in a knit fabric, in the warp than in the other angularly disposed elements, attained either by putting in more ends of rubber, or by using heavier rubbers, to give more resistance to stretching warpwise than transversely. But because the same rubber cord will contract more strongly when stretched to near the limit of its extensibility than it will at the beginning of its stretch, starting from fully or nearly contracted relation, an important feature of the invention provides for inserting the

70

75

80

85

90

95

100

105

110

115

120

125

130

elastic warps in the woven fabric in substantially completely expanded relationship, stretched as close to the breaking point as is safe, while putting in the elastic wefts under 5 a tension which leaves them far short of their full extension. Thus, other things being equal, an equal number of identical warps and wefts per inch put in in accordance with this phase of the invention can be made to 10 give a greatly preponderant force of contraction to the fabric in the direction of the warps. The insertion of non-elastic wefts along with the elastic wefts, while these latter are being put in at well under maximum tension, 15 perpetuates the relationship thus established through preventing weftwise strains on the fabric from stretching the elastic wefts far enough to run up their tensions to a degree comparable with those of the elastic warps. 20

Thus I prefer to use non-elastic weft along with the elastic weft. If all the picks be made elastic, and inserted in sufficient numbers to give the fabric the required body, the 25 contractive power of these wefts is apt to be so great, even when the fine rubber cords just indicated are used as weft, as to overcome the friction of the marginal portions of the fabric against the underlying surfaces, making 30 the fabric slip instead of stretching as the wearer bends over, unless an unusually rough frictional surface be provided on the fabric, which latter narrows the field of the fabric's utility. The fibrous wefts make possible 35 an exact and easy proportioning of the weftwise contractive power of the fabric to the warpwise contractive power, because they can be added or reduced in number to complement the reduction or addition of the rubber wefts, while keeping the density of the 40 fabric as desired. Thus the presence of the fibrous wefts is important both as regards the rubber warps and as regards the rubber wefts, because by diluting the concentration of the 45 rubber wefts it facilitates the obtaining of any desired ratio between the lengthwise and transverse contractive effects, thus avoiding on the one hand difficulties arising through 50 too great or too slight weft density, and on the other the awkward necessity of changing the tension under which the elastic wefts are inserted.

In the accompanying drawings,—

Fig. 1 is a more or less diagrammatical 55 representation of one face of a fabric having both lengthwise and transverse stretch, integrally combined in the weaving with portions having extensibility only in the direction of their length.

Fig. 2 is a similar diagrammatical representation of a section on line 2—2 of Fig. 1, at right angles to the warps, with the fiber wefts omitted for clarity.

Figs. 3 and 4 show leno fabrics, longitudinally extensible, which are rendered capable

of simultaneous transverse stretch through the use of elastic wefts in accordance with the invention.

Figs. 5 and 6 show other leno fabrics including both elastic warp and elastic weft, and hence extensible simultaneously both warpwise and weftwise in accordance with the invention.

Fig. 7 shows a fabric in which elastic warps are combined with elastic and non-elastic wefts without interweaving, by the use of straight-woven face and back non-elastic binder warps.

Fig. 8 shows a typical girdle, the component fabric of which, indicated at *a* may be any one of the invention fabrics of the foregoing figures.

The embodiment shown in Figs. 1 and 2 illustrates the novel fabric as made by weaving, and integrally combined with portions of woven fabric having stretch only in the direction of their length, a combination having obvious desirable features for use in the manufacture of girdles and corsets. Thus, the central portion of the width of the fabric 85 extending from B to C comprises the novel elastic fabric having capacity for stretching simultaneously both in the direction of its length and of its width, or "two-way stretch", while the flanking portions of the width of the integral fabric which extend from A to B and from C to D are capable of being stretched only in the direction of their length, and thus have "one-way stretch".

The particular embodiment of Figs. 1 and 100 2 comprises elastic warps 1, which may be of any suitable construction, such as the usual vulcanized elastic rubber strands or cords, covered in well-known manner with fibrous wrappings made of several plies of suitable yarn. Between each pair of rubber warps 1 are fibrous non-elastic warps 3, three of which are used between each pair of elastic warps in the one-way stretch fabric, and two of which are employed between each pair of elastic warps in the intermediate two-way stretch portion, the reduction in the number of fibrous warps in the two-way stretch portion being to compensate for the increased body otherwise resulting from the insertion 115 of the elastic weft in this portion, as will be described. Face and back fibrous non-elastic wefts 5, 6, are interwoven with the warps 3 in any desired manner depending on the character or figure desired to be produced 120 on the face and back, and in the weave shown result in the production of a face and back having identical appearance, a feature of advantage in certain uses to which the fabric may be put, as where the garment is desired to be made reversible. The face and back wefts 5, 6, are not interwoven with the individual elastic warps 1, being pressed tightly enough against the face and back surfaces

125 of the warps 1 through the action of the 130

fibrous binder warps 3 to maintain the elastic warps 1 against slipping in the fabric even though these warps 1 are woven under tension. The face wefts 5 after traversing the 5 one-way stretch portion pass to the back of the fabric at the line B joining the marginal one-way stretch portion with the central two-way stretch portion, changing just outward of the warp 1<sup>b</sup>, and lying at the back 10 across the full width of the two-way stretch portion and returning to the face over the elastic warp 1<sup>a</sup> adjacent the line C at the right-hand edge of the two-way stretch portion, remaining at the face across the other 15 portion having one-way stretch extending from C to D, or to the selvage of this latter portion, as will be understood. The back wefts 6 similarly change to the face at the line B, and return to the back just before 20 they reach elastic warp 1<sup>a</sup>. The practice of the invention being in no way dependent on the particular method of working these wefts, it is to be understood that this is merely one satisfactory way of doing so, and is 25 not restrictive.

The novel elastic weft 7 is inserted in the fabric from line B to line C to form the two-way stretch portion, herein being interwoven with the elastic warps 1 across the interval, 30 and it may likewise be interwoven with the fibrous warps 3 in any suitable or desired manner. The material of this elastic weft 7 may be any known rubber cord, preferably covered, of suitable character, such as that 35 of the Adamson patent aforesaid. It is desired that the uncovered rubber core itself be of relatively small diameter, and an indication of the proper size is that it should be substantially commensurate in diameter with 40 the non-elastic fibrous warps 3 which will be used in the fabric; in other words, the core of the rubber cord will normally range from No. 50 (1/50 of an inch in diameter) through various smaller sizes. It is found 45 that larger wefts, being stronger, have to be separated farther apart from each other in the fabric, in order to make the fabric gentle enough in its transverse stretch to have the proper ratio to its lengthwise stretch, and 50 this excessive spacing of the wefts, with the requisite filling-in of non-elastic wefts to give body, tends to make the intermediate areas of the latter shirred and uneven when the rubber warps contract and gather them, 55 also forming transverse ribs where the rubber wefts are. Such a fabric becomes unsuitable for use as an undergarment, as too rough to go against or close to the skin.

Elastic wefts of the sizes indicated, being 60 fine, are weak, and the successive picks can be put much closer together without making the fabric too strong and without loss of the desired contraction ratio aforesaid, even when the non-elastic wefts are eliminated 65 entirely; though where used, the reduced

number of intervening non-elastic wefts makes possible the controlled and nearly invisible gathering or shirring of these wefts, and the rubber weft cords being smaller in diameter there are no transverse ribs. The 70 result is a smooth surfaced fabric eminently suitable to go against the skin.

It is essential that the fabric shall lie flat, and not tend to curl or roll up, when taken from the loom, otherwise the fabric has little 75 or no commercial value. This requirement, more difficult of attainment in a two-way stretch fabric than in the previous one-way stretch materials, has been met in accordance with the invention through balancing the 80 amount of rubber at one face by an equal amount at the other, both as regards the rubber warp and as concerns the rubber weft; and through preferably always inserting two elastic picks side by side in directly opposed 85 relation, these successive picks work directly against each other and cancel each other's tendency to curl the fabric, even though a number of non-elastic wefts precede and follow each pair.

The elastic weft is preferably inserted under a tension sufficient with regard to the various factors to produce the widthwise contraction of the fabric when taken from the loom which is to bring the garment fashioned 90 therefrom back into shape as the wearer straightens up, without causing slipping of the margins of the garment when the wearer bends. This weft tension is of appreciable extent and easily ascertained by one skilled 95 in the art; it is of totally different and lesser degree from the tension under which the elastic warps are inserted. These latter are pulled out practically to the limit of their stretch, while the elastic wefts, on the other hand, are preferably merely at the beginning 100 instead of at the limit of their stretch as inserted, this moderate degree of tension being easily achieved by tension devices in the shuttle.

The non-elastic or fibrous wefts 5, 6, act in another way to create and preserve the proper working ratio between the lengthwise and transverse contractibility, through compelling 110 the elastic wefts to operate within a narrow range of relatively gentle tensions at the beginning of their stretch. In this and the other fabrics of the invention the elastic wefts because put in under tension, are normally shorter than the non-elastic weft elements, 115 but they are not drawn out to the limit of their stretch at the time when they are put in; hence the fibrous wefts 5, 6, prevent the rubber wefts from ever being stretched beyond the moderate tension at which inserted, 120 and therefore prevent the contractive effort of the elastic wefts from reaching anywhere near their maximum because the fibrous wefts limit the stretch long before the elastic elements have reached the limit of their exten- 125 130

sion. It is to be noted that in each instance illustrated a fibrous weft lies adjacent each elastic weft element, at one side or the other thereof. Thus is attained an effect similar 5 and closely equivalent to that which is made possible in weaving certain elastic fabrics by running a slack rubber warp with a tight fibrous warp wrapped around it through the same eye in the harness and the same dent 10 in the reed as disclosed in Patents Nos. 1,566, 727, and 1,577,728, granted on Dec. 22, 1925, to F. L. Brigham; as there, I insert a pick of rubber weft which is not extended to its full stretch, and insert alongside of it a stretch- 15 limiting non-elastic weft. The non-elastic weft of course has the same effect as the non-elastic stretch-limiting warps just described in prolonging the life of the elastic through preventing its being strained to the limit, as 20 well as serving the additional ends of diluting the concentration of rubber extending weftwise in a given length and of holding the rubber weft down to the weak end of its stretch.

25 In the specific form of Figs. 1 and 2 the elastic weft is inserted under moderate tension in two successive and adjacent picks, which are worked exactly opposite. There- 5. 6. 30 after, four picks of face and back wefts are inserted, and then two more picks of the elastic weft are put in. The arrangement shown at the right hand terminus of the two- 35 way stretch central portion is particularly suited for use in a light and flexible fabric, the elastic weft 7 being looped around and forming its reverse bend through engage- 40 ment with the elastic warp 1<sup>a</sup> which lies just outward of the crossing of the face and back wefts 5 from one surface to the other of the fabric, as shown in Fig. 1; by such crossing, as well as by its own tension at all times, this warp 1<sup>a</sup> is effectually held from being pulled inward through the contraction of the elastic weft with accompanying distortion of the de- 45 sired flat aspect of the fabric. As shown, the portion of the continuous elastic weft 7 which extends between one group of two picks and the next similar group is simply floated over all the wefts until it again reenters the fab- 50 ric, looping around elastic warp 1<sup>b</sup>; because the four picks of face and back wefts 5, 6, pack together closely, the float is of incon- 55 spicuous length and aspect, and elastic warp 1<sup>b</sup>, being always tense, prevents distortion of the fabric.

Ordinarily, the two-way stretch fabric as shown between the lines B and C may be woven as a single homogeneous material. But peculiar advantages flow from the com- 60 bination of the two-way stretch fabric with flanking sections of one-way stretch elastic fabric, where the material is to be used as contemplated for corsets and girdles, where the aim is to prevent the top and bottom 65 margins of such a garment from slipping

and changing their position on the wearer's body when the latter is flexed. Thus, it is contemplated within the scope of the present invention to combine the two materials, the old and the new, either through weaving the 70 two materials separately and thereafter combining them by sewing or otherwise uniting the selvages of the two materials together, or preferably as indicated in Fig. 1, through weaving them integrally in one piece and 75 with component elements common to both, as shown and described. Made in either way, the one-way stretch cuff flanking the top and bottom edges of the two-way stretch portion as the fabric is utilized in a girdle possesses 80 a rigidity and freedom from yield or stretch up and down the wearer's body which definitely grips the underlying surfaces and serves to belt the top and bottom of the garment to definite points on the wearer's body above the hip bones and below the hips, and to fix the position of these portions of the garment, while the intermediate two-way 85 stretch portion spreads and recovers as the underlying portions of the body become 90 convex or concave; and further provides a rigid band at the bottom of the garment for sewing the garters to. The invention fabric enables the maker of such corsets and garters and similar garments easily to define the 95 waist line of the wearer and to define it in such a way as not to impede the movements nor interfere with the comfort of the wearer, while the vertical strains on the garment, re- 100 sulting from a sitting posture of the wearer, are relieved through the presence of the two- way stretch material across the back of the garment, resulting in prolonged life and 105 utility of the garment.

Figs. 3 and 4 show the invention principles applied to produce two-way stretch elastic fabrics through the use of leno or cross- weaving. In Fig. 3, the covered rubber warps 9 are combined with the rubber wefts 11, 13, and the non-elastic or fibrous wefts 15, 17, without interweaving; a non-elastic leno warp 19, 21, being associated with each rubber warp 9 and crossing back and forth over its rubber warp at one surface of the fabric to engage beneath a pair of elements comprising a fibrous weft 17 and an elastic weft 11 lying at the back of the fabric. In its crossing, it binds a face elastic weft 13 and a face fibrous weft 15 against its proper elastic warp 9. Each two adjacent leno warps are run symmetrically with respect to each other, converging and diverging and crossing their respective warps with opposite inclination, as plain in Fig. 3. In Fig. 4, 110 the construction is identical, except that the leno warps 23 are all run parallel to each other, the difference resulting in giving the fabric of Fig. 3, a slight reticulated or honey- 115 comb aspect, while that of Fig. 4 has a dis- 120 tinctly ribbed or twilled appearance. In 125 130

each of these fabrics, the crossing of the rubber warps by the lenos has been found to impart to the surface shown in the drawings just enough friction to cling to the skin of the wearer without being too rough and uncomfortable. Another feature of the fabrics of Figs. 3 and 4 is that the weft, both elastic and non-elastic, need not be interwoven with the warps, but runs straight and without perceptible undulation in two separate planes above and below the elastic warps. This is of considerable advantage in giving to the fabric a flat and level surface at each face. While the fabric of Figs. 1 and 2 is characterized by longitudinal ribs at both surfaces, the surface of the fabric shown in Fig. 3 though reticulated is notably more level and totally devoid of longitudinal ribs, while that of Fig. 4 has low transverse ribs which present a flatter and more level surface than the construction of Fig. 1. The other advantages attained in the fabric of Fig. 1 are secured in even greater measure, for the elastic wefts are inserted in adjacent pairs at opposite faces of the fabric, and through being run without interweaving are easily balanced in tension, one against the other, to make a fabric that will lie flat; while the fibrous wefts 15, 17, which thin out the elastic wefts are even more intimately associated each with its adjacent elastic weft by the binding action of the leno, so as even more completely to allow the insertion of the elastic weft with any desired degree of minimum tension, without allowing the strain of weft-wise expansion of the fabric to run up the tension and resulting contractive force of the elastic wefts, much less allow these elastic wefts to be strained to their limit.

Fig. 5 shows another form of two-way stretch leno fabric related to that shown in Fig. 4, having in addition to the elements and arrangements of Fig. 4 a non-elastic fibrous warp 25 associated with each elastic warp 9, and worked the same way as its proper elastic warp with respect to the elastic wefts 11, 13, but oppositely to the elastic warps with respect to the non-elastic wefts 15, 17. The fibrous warps 25 are included within the crossings of the parallel lenos associated with each elastic warp 9. The result is a fabric with a face having transverse ribs of which alternate ones are conspicuous and intermediate ones are not noticed, owing to the changing slant of the lenos; while the back is notably smoother than in the other examples owing to the presence of the fibrous warp 25.

In Fig. 6, the elastic wefts are paired and opposed at opposite faces of the fabric without interweaving with the warps, as described. Two fibrous warps 27, 29, are associated with each elastic warp 9, while two leno warps cooperate with each group of elastic and non-elastic warps, instead of one, as in the prior examples. The fibrous warps 29 engage under two picks and over every third, whether rubber or fiber, while the intermediate fibrous warps 27 engage under five picks and over the sixth; they are properly back warps and impart softness and smoothness to the back. Four picks of non-elastic weft, 31, 32, 33, 34, are interposed between each successive pair of elastic wefts 35, 36, of which three lie at the back of the elastic warps for every one at the face. The face leno 37 crosses back and forth over its rubber warp 9 between the points where the face picks of elastic weft 35 and non-elastic weft 34 are laid across, so that these wefts are not stitched into the fabric by this leno, but instead are held to the warps by the back leno 39, which passes over these two wefts from behind, crossing over the back elastic wefts 36 and their associated fibrous wefts 31 where these two intersect the rubber warps 9, and engaging over the same pick of fibrous back weft 32 under which is engaged the face leno 37. Each rubber warp has two fibrous warps 27, 29, associated with it, and included within the zigzags of its proper face and back lenos. It is to be noted that the face and back lenos both pass from one face of the fabric to the other at the same time; this makes a crossing of these warps which spreads apart the wefts immediately preceding and following such crossing. Since this crossing occurs after every other pick and occasionally both before and after a single pick, the fabric is given an openwork texture which makes it porous and well ventilated when in use as a garment. Since the face leno does not cross at the points where the face wefts cross the warps, the face of the fabric is given a rectangular reticulated aspect differing from the diagonal honeycomb appearance of Fig. 3, as the face leno does not clip the corners of the squares defined by the warps and wefts. The back of the fabric is exceedingly soft and smooth, owing to the long floats of the fibrous warps 29 and the additional fibrous back wefts 32 and 33.

Fig. 7 shows a straight weave in which the elastic warps 9 are likewise not interwoven with the elastic wefts 41, 43, but establish the latter in face and back weft planes. The elastic wefts are each accompanied by adjacent fibrous wefts 45, 47, respectively, worked the same way as their respective elastic wefts, and the wefts are bound to the elastic warps by fibrous warps 49, 51, which are worked in a warp twill weave, passing under a back elastic weft 43 and its associated back fibrous weft 47 and thereafter floating for six picks at the surface. The face and back of the fabric are identical, as the back warps 51 are worked in similar manner.

While I have illustrated and described certain forms in which the invention may be embodied, I am aware that many modifications

tions may be made therein by any person skilled in the art, without departing from the scope of the invention as expressed in the claims. Therefore, I do not wish to be limited to the particular forms shown, or to the details of construction thereof, but

What I do claim is:—

1. In a corset, girdle, or the like supporting garment, elastic fabric having in combination parallelly extending elastic elements, and other elastic elements extending intermediate each adjacent pair of the first elements in angular relation to the latter, one of the two sets of elastic elements being capable of exerting a strong contractive effort and the other restricted to a contractive effort materially below that of the first set as the garment is worn. 10
2. In a corset, girdle, or the like supporting garment, woven elastic fabric having in combination a set of elastic rubber warp elements, and a set of elastic rubber weft elements, one of such sets of elastic elements arranged to exert a contractive effort materially below that of the other as regards portions of the fabric of equivalent size. 20
3. In a corset, girdle, or the like supporting garment, woven elastic fabric having in combination elastic rubber warp elements, elastic rubber weft elements, non-elastic yarns limiting the stretch of the elastic warps at or about the maximum extensibility of the latter, and non-elastic yarns preventing the stretch of the elastic wefts beyond a fraction of their normal extensibility. 30
4. In a corset, girdle, or the like supporting garment, elastic fabric having component elements of rubber permitting simultaneous stretching of the garment in two dimensions through elongation of the rubber elements, the contractive force of the elastic fabric in the garment being materially greater in one of such dimensions than in the other, under like conditions. 40
5. In a corset, girdle, or the like supporting garment, woven elastic fabric having in combination elastic warp elements, non-elastic weft elements coextensive with the width of the fabric, and elastic weft elements interspersed with the non-elastic wefts and terminating short of the full width of the fabric. 50
6. Woven elastic fabric having in combination elastic warps, elastic and non-elastic wefts crossing the elastic warps without interweaving therewith, and non-elastic warps binding a pair of adjacent wefts, comprising an elastic weft and a non-elastic weft, to the elastic warps alternately at one face and then at the other of the fabric, the elastic wefts being inserted in adjacent pairs. 60
7. Woven elastic fabric having in combination elastic warps, face and back elastic wefts, face and back non-elastic wefts, and leno warps engaging first a face elastic weft, and a face non-elastic weft, and then a back elastic weft and a back non-elastic weft, the elastic wefts being inserted in adjacent pairs. 70
8. In a corset, girdle, or the like supporting garment, elastic fabric capable of being stretched as a whole in the direction of its length, and having a portion of its width capable of being simultaneously stretched transversely, and another portion of its width incapable of transverse stretch. 75
9. In a corset, girdle, or the like supporting garment, elastic fabric comprising in combination one or more marginal portions capable of being stretched lengthwise only and an intermediate portion capable of being stretched simultaneously both lengthwise and crosswise. 80
10. A corset, girdle, or the like supporting garment including in its composition an elastic fabric having in combination a set of elastic and non-elastic warps, and a set of elastic and non-elastic wefts, the stretch of the fabric in the direction of one of these sets of elements being limited to less than the stretch in the direction of the other set. 85
11. In a corset, girdle, or the like supporting garment, woven elastic fabric having in combination elastic warps distributed across substantially the full width of the fabric, and elastic wefts inserted in groups of one or more pairs of oppositely-worked adjacent picks each of which picks in a pair substantially balances the tendency of the other pick to curl the fabric, with the groups separated by one or more picks of non-elastic weft, and with the elastic weft less in extent than the width of the fabric. 90

THOMAS F. MOORE.

105

110

115

120

125

130

CERTIFICATE OF CORRECTION.

Patent No. 1,896,783.

February 7, 1933.

THOMAS F. MOORE.

It is hereby certified that error appears in the printed specification of the above numbered patent requiring correction as follows: In the drawings, sheet 2, at the right hand side, strike out "Fig. 8," showing a fabric weave; and that the said Letters Patent should be read with this correction therein that the same may conform to the record of the case in the Patent Office.

Signed and sealed this 28th day of February, A. D. 1933.

(Seal)

M. J. Moore,  
Acting Commissioner of Patents.

## DISCLAIMER

1,896,783.—*Thomas F. Moore*, Westerly, R. I. ELASTIC FABRIC. Patent dated February 7, 1933. Disclaimer filed August 4, 1933, by the assignee, *George C. Moore Company*, the patentee, said Moore, approving and ratifying.

Hereby enters this disclaimer to that part of the claim in said specification which is in the following words, to wit:

“4. In a corset, girdle, or the like supporting garment, elastic fabric having component elements of rubber permitting simultaneous stretching of the garment in two dimensions through elongation of the rubber elements, the contractive force of the elastic fabric in the garment being materially greater in one of such dimensions than in the other, under like conditions.”

[*Official Gazette August 29, 1933.*]